

July 20, 1971

R. G. CHARLES ET AL

3,594,216

VAPOR PHASE DEPOSITION OF METAL FROM A METAL-ORGANIC  
BETA-KETOAMINE CHELATE

Filed June 19, 1969

2 Sheets-Sheet 1



FIG. 1.



FIG. 3.

WITNESSES

Theodore G. Wrobel  
Daniel P. Cillo

INVENTORS

Robert G. Charles  
and James G. Cleary  
BY Alex Mich Jr.

ATTORNEY

July 20, 1971

R. G. CHARLES ET AL

3,594,216

VAPOR PHASE DEPOSITION OF METAL FROM A METAL-ORGANIC  
BETA-KETOAMINE CHELATE

Filed June 19, 1969

2 Sheets-Sheet 2



FIG. 2.

3,594,216

## VAPOR PHASE DEPOSITION OF METAL FROM A METAL-ORGANIC BETA-KETOAMINE CHELATE

Robert G. Charles, Allison Park, and James G. Cleary, Pittsburgh, Pa., assignors to Westinghouse Electric Corporation, Pittsburgh, Pa.

 Filed June 19, 1969, Ser. No. 834,642  
 Int. Cl. C23c 11/02

U.S. Cl. 117—107.2

6 Claims

### ABSTRACT OF THE DISCLOSURE

A metallic coating is deposited on a substrate by heating the substrate and contacting the substrate with vaporized metal-organic beta-ketoamine chelates, which react on contact with the hot substrate surface in a gaseous atmosphere to deposit the metal coatings.

### BACKGROUND OF THE INVENTION

This invention relates to the vapor phase deposition of metallic substances from certain metal chelates.

Chemical vapor-deposition coating methods were developed from techniques employed as early as 1880 by the incandescent lamp industry. A few years later, attention was directed to vapor deposition as a method of preparing high purity metals.

Chemical vapor deposition is a method of plating in which the deposits are produced by heterogeneous gas-solid or gas-liquid chemical reactions at the surface of a substrate. A volatile compound of the element or substance to be deposited is vaporized and the vapor thermally decomposed, or reacted with other gases or vapors, at the substrate to yield nonvolatile reaction products which deposit on the substrate as a coating.

Nickel has most usually been deposited from the vapor phase by the thermal decomposition of nickel tetracarbonyl,  $\text{Ni}(\text{CO})_4$ . This procedure, through nickel tetracarbonyl decomposes at inconveniently low temperatures for some purposes, seems to be quite satisfactory in terms of the nickel films obtained. Nickel tetracarbonyl is, however, highly toxic-sufficiently so to discourage its use despite its other advantages. It is desirable therefore to find alternative volatile metal compounds, from which satisfactory metallic films or coatings can be obtained, and which avoid this toxicity hazard. Nickel acetylacetone:



has been tried, but seems to require reduced pressure for optimum results and suffers from premature thermal decomposition. Nickel hexafluoroacetylacetone and nickel trifluoroacetylacetone have also been tried, but they are quite expensive to prepare.

### SUMMARY OF THE INVENTION

Accordingly, it is an object of this invention to provide improved and inexpensive plating compounds suitable for vapor phase deposition of various metals.

It is a further object of this invention to provide a new and improved process for the vapor phase deposition of nickel and other metals or combinations of metals from metal organic beta-ketoamine chelates.

Briefly, the above objects are accomplished in accordance with the present invention, by (1) vaporizing metal organic beta-ketoamine chelates, for example: nickel acetylacetone imide, copper acetylacetone imide, bisacetylacetoneethylenediiimine nickel, and bisacetylacetoneethylenediiimino copper, in a porcelain or silica boat container within a cylindrical quartz furnace tube at pressures up

to and including atmospheric; (2) causing the vaporized metal chelate to be carried by pure hydrogen gas to a platinum, quartz or a glass fiber target substrate, held at a controlled temperature substantially higher than the vaporization temperature of the metal chelate, so as to deposit a pure metal coating on the substrate through hydrogen reduction of the chelate; (3) exhausting deposition by products for safety, and a possible recycling procedure.

The nickel and copper acetylacetone imides have a high degree of volatility, are relatively nontoxic, and comparatively easy and inexpensive to prepare. The nickel and copper acetylacetoneethylenediiimides also have definite advantages in terms of cost, ease of preparation and ease of handling these compounds can yield pure, dense, adherent metal coatings for a variety of end uses such as growing films on chosen substrates for molecular electronic devices, or coatings or structures of refractory materials for use in the aerospace industry.

Further objects and advantages of the invention will become apparent as the following description proceeds and features of novelty which characterize the invention will be pointed out in particularity in the claims annexed to and forming a part of this specification.

### BRIEF DESCRIPTION OF THE DRAWINGS

For a better understanding of our invention, reference may be had to the accompanying drawings, in which:

FIG. 1 shows a simplified schematic drawing of the vapor-desposition process;

FIG. 2 shows a flow diagram for vapor deposition; and

FIG. 3 shows a sectioned view of the deposition apparatus used in the experiments.

### DESCRIPTION OF THE PREFERRED EMBODIMENTS

The preferred metal-organic beta-ketoamine chelates for use as suitable volatile starting materials for the chemical vapor deposition of their respective metals, are chelates of the following structures:

#### 40 (STRUCTURE I)



wherein M can be Ni, Cu, Co, and Cr among other metals,  $R_1$  can be  $\text{CH}_3$  or  $\text{CF}_3$ ,  $R_2$  can be  $\text{CH}_3$  or  $\text{CF}_3$ ,  $R_3$  can be  $\text{H}$ ,  $\text{CH}_3$  or  $\text{CF}_3$  and X can be  $\text{H}$  or  $\text{CH}_3$ , and

#### 40 (STRUCTURE II)



wherein M can be Ni and Cu among other metals,  $R_4$  can be  $\text{CH}_3$  or  $\text{CF}_3$ ,  $R_6$  can be  $\text{CH}_3$  or  $\text{CF}_3$ ,  $R_6$  can be  $\text{H}$ ,  $\text{CH}_3$  or  $\text{CF}_3$  and X can be  $\text{H}$  or  $\text{CH}_3$ . Best results have been achieved with nickel acetylacetone imide (bisacetylacetoneimide nickel (II))



as an example of Structure I, and with copper and nickel acetylacetoneethylenediiimides (bisacetylacetoneethylen-

diimine copper (II) and nickel (II) as examples of Structure II:



Although Ni, Cu, and Co are the preferred metals, other metals that are also considered within the scope of this invention include Fe, Mn, Cr, Pd, and Pt as well as mixtures of all these metals to form alloys of Fe, Co, Cu, Ni, and Cr. These alloys might be deposited by co-deposition of several different metal-organic beta-ketoamine chelates.

The following preferred procedure can be used to yield nickel acetylacetone imide (bisacetylacetoneimide nickel (II) also bis 4-imino-2-pentanone-nickel (II) one of the metal-organic beta-ketoamine chelates which we used as a metal vapor deposition plating compound in this invention (Structure I): to a solution of acetylacetone imide (4-imino-2-pentanone) in ethanol is added a solution of nickel (II) nitrate 6-hydrate in water containing aqueous ammonia. The reaction mixture is shaken vigorously and allowed to stand. The precipitate forms as follows:



Other chelates of Structure I can be formed analogously by mixing an ethanolic solution of the beta-keto imine (beta-imino ketone) with an ammoniacal metal salt solution.

The following preferred procedure can be used to yield nickel acetylacetoneethylenediimide (bisacetylacetoneethylenediimino nickel (II)), another of the metal-organic beta-ketoamine chelates which we used as a metal vapor deposition plating compound in this invention (Structure II): to a solution of recrystallized bisacetylacetoneethylenediimine is added an aqueous solution of nickel acetate tetrahydrate. To that mixture aqueous ammonia is added and the reaction mixture heated nearly to boiling. The precipitate forms after the reaction mixture is cooled. Copper acetylacetoneethylenediimide can be prepared by substituting copper acetate monohydrate for nickel acetate tetrahydrate in the method above.

The chemical vapor-deposition processes constitute a highly versatile and flexible means of applying a coating of most of the refractory metals and nonmetals. Coating thickness can be varied, and fairly well controlled over a wide range, and most refractory materials can be obtained in a purer state by vapor-deposition processes, than by conventional metallurgical practices.

One of the most frequently used types of chemical vapor-deposition reaction is hydrogen reduction, at an elevated temperature, of the plating compound vapor. Hydrogen reduction is carried out at elevated temperatures where the reduction reaction is favored because a favorable thermodynamic equilibrium or a suitably rapid reaction rate is attained. Hydrogen reduction may be thought of as a thermal decomposition reaction which is facilitated by removal of one or more of the gaseous products of the decomposition. Consequently, the temperature required for a given extent of decomposition or rate of deposition from a given compound is appreciably lowered, usually by several hundred degrees, below that needed in the absence of hydrogen. It is desirable, in the hydrogen-reduction process, that the plating compound used have appreciable volatility at temperatures well below those at which the reduction reaction is thermodynamically or kinetically favored. If this condition cannot be met, the plating compound will have to be vaporized into a stream of inert carrier gas, which is then mixed with hydrogen at the point or region where deposition is desired.

Referring now to FIG. 1 of the drawings, a metal organic compound 1 (represented in block form) is shown

in a container 2 at a temperature T. Chemically reactive hydrogen gas atoms 3 are shown as well as impurity nitrogen gas atoms 4. The target substrate 5 at a temperature T' has metal atoms 6 deposited or plated on it while the other gaseous byproducts of the decomposition 7 are exhausted or removed through opening 8. In the vapor deposition process shown schematically in FIG. 1, the metal organic is vaporized at a temperature T and carried past the target by hydrogen gas. The metal organic vapor and hydrogen gas mixture come in contact with the substrate 5 at a temperature T', which is lower than the melting point of the metal to be plated but higher than T, and at that point, the hydrogen reduces the metal organic to the metal that is deposited on the hot target.

The advantages of vapor-deposition technology should be obvious after considering the details of the process. It is possible to selectively volatilize a feed material, transport it to a desired location, and precipitate it as a controlled structure. Further details of the thermodynamics, evaporation and transport processes, and nucleation of vapor deposited materials in vapor deposition processes can be found in Powell, Vapor Deposition, John Wiley & Sons, 1966 Chapter 1, herein incorporated by reference.

A flow diagram of the experimental apparatus used in Examples 4, 5, 6, 7, 9, 12 and 14 of this specification is shown in FIG. 2. The hydrogen 20 and argon 21 gases are high purity (99.95%) grade with N<sub>2</sub> and O<sub>2</sub> as the main impurities. The hydrogen is passed over a palladium deoxy catalyst 22, through a CaSO<sub>4</sub> drier 23, then over a molecular sieve and metered at the entrance of the vaporization and plating chamber (deposition apparatus) 24, shown in detail in FIG. 3. The argon gas, if it is to be used, is passed through zirconium turnings 25 heated to 800 degree C. then metered into the plating chamber. Exhaust gases are passed through a Dry Ice trichloroethylene trap, to condense the reaction vapors. A mechanical vacuum pump 26 is used when operating at low pressure.

A sectioned view of the deposition apparatus or plating chamber 24, used in Examples 4, 5, 6, 7, 9, 12 and 14 of this specification is shown in FIG. 3. An external heater 30 surrounds the glass volatilization chamber 31. An inner glass tube 32 supports the sample boat container 33 and is necked down around the target substrate 34 to collimate the sample vapors, thus increasing compound vapor to substrate contact. The target substrate 34 is in good thermal contact with a Kovar metal probe 35 which is heated internally with a Chromalox heater. The metal probe is drilled to accept a thermocouple. In cases where the target temperature goes above 700 degrees C., an alternate target is used consisting of a platinum coil heated resistively with the apparent temperature determined by using a Pyrometer Instrument Company micro-optical pyrometer, Model No. 95-EA5.

In the examples, the metal organics, usually solid, were placed in a silica sample boat and placed into the apparatus rapidly to reduce atmospheric contamination. The carrier gas used was hydrogen. The hydrogen gas flow, through gas inlet 36, was metered into the system through a Hoke vacuum needle valve. This valve permitted complete evacuation of the plating system. The gas flow passed over the sample boat. The vapors of the metal-organic beta-ketoamine chelates were carried along with the carrier hydrogen reducing gas, with reduction occurring at the hot target substrate. Exhaust of the gaseous products of the decomposition was through outlet 37.

Quartz, glass fibers, tantalum and platinum were tried as target substrate materials. The quartz targets used in the examples were tubular cylinders approximately 3/4" x 1 1/4" and closed at one end. The fit of these cylinders was such that good thermal contact was maintained against the Kovar metal probe, providing excellent heat transfer to the target surface. The tantalum and platinum targets were made of 0.008 inch wire wound into coil filaments approximately 1/2 inch long with a coil diameter of 1/8 inch. Temperature control of the target probe was

accomplished using a Wheeler controller with a Chromel-alumel thermocouple. The target filaments were held at temperature by passing an alternating current through the wire coil. The volatilization chamber was heated externally by a split tube furnace with the temperature controlled using a thermoelectric controller with a Chromel-alumel thermocouple. The internal pressure of the system was determined using a thermocouple vacuum gauge and a Wallace-Tierney direct reading dial gauge. In all the following examples this experimental apparatus was used, in conjunction with the hereinafter described procedure.

The plating process of Examples 4, 5, 6, 7, 9, 12 and 14 of this specification was accomplished by the following procedure. After placing the silica boat containing the metalorganic beta-ketoamine chelate (about 200 mg.) into position in the plating chamber 24 shown in FIG. 3 of the drawings, the system was closed by insertion of the target holding end 38 into the glass volatilization chamber 31. A trap was attached at the exhaust gas outlet 37, (cooled using a Dry Ice trichloroethylene bath) then valved to the mechanical pump which evacuated the system. In cases where runs were carried out at atmospheric pressure, the system pressure was then raised and use of the vacuum pump discontinued.

After the system was evacuated, purged and the pressure regulated, the degreased and cleaned target substrate was heated to the desired operating temperature. The hydrogen gas flow was adjusted and the plating chamber heated to the desired temperature of metal plating compound volatilization. The temperature was increased in the final moments of operation to insure the complete volatilization of the sample. The chamber was then cooled while keeping the target at temperature until all the volatile materials were reacted or condensed. The target temperature was then lowered.

After cooling to room temperature, the apparatus was disassembled and the target weighted and inspected visually under a microscope to determine the nature of any deposit. An X-ray diffraction powder pattern of the deposit was then obtained using a 114.6 mm. camera and CuK alpha radiation with a nickel filter. The diffraction unit used was a North American Phillips type 12045/3. In some cases, additional information was obtained by a spectrographic technique using an Associated Electrical Industries MS-702 spark source mass spectrometer. Some film deposits were also examined using an electron diffraction unit with an excitation voltage of 50,000 ev.

The purity of metals deposited from metal-organics and the stoichiometry of compound deposits are influenced by the temperature of the substrate, the vaporizer, system pressure, gas flow, plating compound concentration, and length of time in the deposition zone. Varying these parameters may not only change the appearance of a deposit but completely change its composition. Operation at a reduced pressure to improve uniformity of a deposit may lead to a change in deposit.

#### EXAMPLE 1

The compound Ni-acetylacetoneethylenedimide (bis-acetylacetoneethylenedimino nickel (II)), for use as a metal-organic beta-ketoamine chelate vapor decomposition plating compound, was prepared as follows. Eleven and two-tenths grams (0.05 mole) of recrystallized bis-acetylacetoneethylenedimine, as prepared by the method

of McCarthy, Hovey, Ueno and Martell in J. Am. Chem. Soc. 77, 5820 (1955), was dissolved in 200 ml. of water by gentle heating. To the warm solution was added, slowly with stirring, a solution of 12.4 grams (0.05 mole) of nickel acetate tetrahydrate in 200 ml. of water. One hundred ml. of 1M aqueous NH<sub>3</sub> was then added slowly. The resulting mixture was then heated nearly to boiling, maintained at this temperature for a few minutes, and finally cooled in a refrigerator for several hours. The red crystalline product was filtered off, washed several times with water and air dried to give 10.3 grams of crude product.

The chelate was recrystallized twice by the following procedure. Ten grams of the compound was dissolved in 100 ml. of methanol by gentle heating. The warm solution was filtered and 30 ml. of water added. The mixture was cooled several hours in the refrigerator and the product filtered off, air dried and finally dried for 4 hours at 100 degree C. The recovery was 80% of the crude product taken (M.P. 198-199 degrees C.).

#### EXAMPLE 2

The compound Cu-acetylacetoneethylenedimide (bis-acetylacetoneethylenedimino copper (II)), for use as a metal-organic beta-ketoamine chelate vapor decomposition plating compound, was prepared by essentially the same method as in Example 1. Ten grams (0.05 mole) of copper acetate monohydrate was substituted for the nickel acetate. The yield of crude violet product was 11.1 grams.

The product was twice recrystallized by dissolving in methanol (75 ml. for each 11 grams) by gentle warming. The solution was cooled to room temperature and filtered through filter paper. To the filtrate was added, a little at a time, 75 ml. of water. The mixture was cooled for 2 hours in the refrigerator. The product was filtered off, air dried, and finally dried for 4 hours at 100 degree C. The recovery was 60 to 80% of the amount of crude product taken (M.P. 137-138 degree C.).

#### EXAMPLE 3

The compound Ni-acetylacetone imide (bisacetylacetone imide nickel (II) or bis 4-imino-2-pentanonato-nickel II), for use as a metal-organic beta-ketoamine chelate vapor decomposition plating compound, was prepared as follows. To a solution of 12.0 grams (0.12 mol) of acetylacetone imide in 100 ml. of 95% ethanol was added a solution of 20.4 grams (0.07 mol) of nickel (II) nitrate 6-hydrate in 300 ml. of water containing 25 ml. of 15 M aqueous ammonia. The reaction mixture was shaken vigorously until a light orange precipitate formed. This mixture was allowed to stand approximately 10 hours. After filtration, the 12.0 grams of crude product was recrystallized from 900 ml. of a 1:1 mixture of benzene and petroleum ether (B.P. 90 to 110 degree C.). The first crop of crystals weighed about 8.0 grams. After reducing the volume of the filtrate to 50 ml., of a second crop of 0.60 gram was obtained, (M.P. 349-251 degree C.).

#### EXAMPLE 4

The results of chemical vapor deposition tests, using the aforescribed procedure and the apparatus of FIGS. 2 and 3 of this specification, for Ni-acetylacetoneethylenedimide, as prepared in Example 1, are outlined in Table 1:

TABLE 1

| Compound                                  | Target temp., °C. | Target material | Volatilization temp., °C. | Pressure, torr | Hydrogen flow rates, cc./min. | Remarks                                                                         |
|-------------------------------------------|-------------------|-----------------|---------------------------|----------------|-------------------------------|---------------------------------------------------------------------------------|
| Ni-acetylacetoneethylenedimide (200 mg.). | 450               | Quartz.....     | 232                       | 730            | 75                            | A very light metallic coating was formed, but not enough for X-ray diffraction. |
|                                           | 550               | Pt.....         | 246                       | 730            | 80                            | A nickel deposit was readily formed.                                            |
|                                           | 600               | Pt.....         | 232                       | 730            | 200                           | Nickel was readily deposited.                                                   |

The results indicate that nickel metal may be easily deposited from this compound at the temperatures tested. A target substrate temperature of 450 degree C. gave only a small and scattered coating but at the higher temperatures, a good coating of nickel was readily obtained.

#### EXAMPLE 5

The results of chemical vapor deposition tests, using the aforescribed procedure and the apparatus of FIGS. 2 and 3 of this specification, for Cu-acetylacetoneethylenedimide, as prepared in Example 2, are outlined in Table 2:

TABLE 2

Compound: Cu-acetylacetone-ethylenedimide (200 mg.)

|                               |        |
|-------------------------------|--------|
| Target temp., °C.             | 450    |
| Target material               | quartz |
| Volatilization temp., °C.     | 204    |
| Pressure torr                 | 730    |
| Hydrogen flow rates, cc./min. | 90     |

In this experiment copper metal was successfully plated on the quartz target.

#### EXAMPLE 6

The results of chemical vapor deposition tests, using the aforescribed procedure and the apparatus of FIGS. 2 and 3 of this specification, for nickel-acetylacetone imide, as prepared in Example 3, are outlined in Table 3:

TABLE 3

| Compound                            | Target temp., °C. | Target material  | Volatilization temp., °C. | Pressure, torr | Hydrogen flow rates, cc./min. | Remarks                                                        |
|-------------------------------------|-------------------|------------------|---------------------------|----------------|-------------------------------|----------------------------------------------------------------|
| Nickel acetylacetoneimide (200 mg.) | 250               | Quartz           | 199                       | 730            | 150                           | Nickel and Ni <sub>3</sub> C were formed.                      |
|                                     | 325               | do               | 176                       | 40             | 200                           | Nickel and Ni <sub>3</sub> C were deposited.                   |
|                                     | 300               | do               | 232                       | 730            | 100                           | Nickel was deposited.                                          |
|                                     | 400               | do               | 260                       | 730            | 200                           | Do.                                                            |
|                                     | 400               | Pyrex glass wool | 260                       | 730            | 150                           | Nickel was deposited as a uniform coating on the glass fibers. |

At target temperatures of 300 and 400 degrees C., an excellent coating of pure nickel metal was formed. The coating was bright and metallic in nature. At 250 degrees C., a small amount of Ni<sub>3</sub>C was also deposited along with nickel metal. When the pressure was reduced and the target temperatures held at 325 degrees C., then the predominant deposit was Ni<sub>3</sub>C with small amounts of nickel metal present. All the deposits were smooth and bright. Metal carbide formation would seem to be favored by low pressure and low target temperatures.

In a second set of experiments using an apparatus similar but not exactly identical to that shown in FIG. 3 of the drawings, we were able to determine quantitatively the amount of nickel metal produced from nickel acetylacetone imide as a function of substrate temperature. It was found, for a carrier gas of pure hydrogen at atmospheric pressure, that the yield of nickel metal was essentially quantitative at substrate temperatures above 300 degrees C.

When fine Pyrex Glass Wool fibers (Fisher Scientific Co.) were used as the target in Example 6, those fibers exposed to the hydrogen and nickel acetylacetone imide vapors were found to be coated with a uniform and adherent nickel metal coating. The coated fibers were electrically conductive and were attracted to a permanent magnet. Nickel plated glass or quartz wool prepared in this way may be useful for such applications as electrodes or in other applications where high surface area of nickel metal is desired.

In the deposition examples above, the hydrogen functioned both as a carrier gas for the chelate vapors and also entered into the deposition reaction. The simplest representation for the reduction involves the straight forward

replacement of nickel by hydrogen in the organic portion of the chelate for example, with Ni-acetylacetone imide:



At least a portion of the acetylacetone imide produced appears to undergo further reactions during the nickel deposition reaction. These most likely involve hydrogenation, since the combination of abundant hydrogen, relatively high temperatures, and a freshly deposited and probably catalytically active nickel surface would seem to be ideal for such reaction to occur to produce products such as those shown below.



To demonstrate the actual importance of hydrogen in the nickel deposition reaction we carried out an experiment with nickel acetylacetone imide (target temp. 400

degrees C., volatilization temp. about 260 degrees C., pressure 730 torr) in which 150 cc./min. of high purity helium was substituted for the hydrogen normally used. No appreciable deposition of nickel occurred, while nickel deposits quantitatively under these conditions in hydrogen.

The extent to which one of the gaseous products of decomposition, the chelating agent, acetylacetone imide, is regenerated during nickel deposition may have economic significance, since it could be recycled to form additional nickel acetylacetone imide and hence reduce the overall cost of the process.

The purity of deposits in Examples 4, 5 and 6 were determined by X-ray diffraction using conventional techniques and carbon analysis using a Leco Low Carbon Analyzer.

#### EXAMPLE 7

The results of chemical vapor deposition tests, using the aforescribed procedure and the apparatus of FIGS. 2 and 3 of this specification, for copper acetylacetone imide (prepared by the method of A. Struss and D. Martin in *Inorganic Synthesis* 8, 2 (1966)) are outlined in Table 4 below:

TABLE 4

|                                                |        |
|------------------------------------------------|--------|
| Compound: Copper acetylacetone imide (200 mg.) | 400    |
| Target temp., °C.                              | 400    |
| Target material                                | Quartz |
| Volatilization temp., °C.                      | 287    |
| Pressure, torr                                 | 730    |
| Hydrogen flow rate, cc./min.                   | 150    |

In this experiment copper metal was deposited as a bright mirror coating. It was identified by X-ray diffraction analysis.

**9**  
**EXAMPLE 8**

The compound cobalt (II) acetylacetone imide (bis-acetylacetone imide cobalt (II) or bis-4-imino-2-pentanonato cobalt (II), for use as a metal organic beta-ketoamine chelate vapor deposition plating compound, was prepared as follows. Acetylacetone imide (3.30 grams) and 3.61 grams anhydrous  $\text{CoBr}_2$  were mixed, as solids, in a flask. The mixture was heated briefly on a hot plate until a blue slurry was obtained. After cooling, 1.85 grams of potassium tert-butoxide was stirred in as a solid. After the initial exothermic reaction had subsided, 35 ml. of absolute ethyl alcohol was added and the mixture was heated with stirring until the blue color disappeared and a brown solid formed (about 15 minutes). The mixture was then evaporated to dryness to room temperature in a stream of nitrogen. The brown lumpy residue was washed with successive 25 ml. portions of water and transferred to a sintered glass crucible. Drying in a vacuum gave 1.25 grams of red product having a melting point of about 235 degree C.

**EXAMPLE 9**

The results of chemical vapor deposition tests, using the aforescribed procedure and the apparatus of FIGS. 2 and 3 of this specification, for cobalt (II) acetylacetone imide, as prepared in Example 8, are outlined in Table 5 below:

**TABLE 5**

|                                                     |        |
|-----------------------------------------------------|--------|
| Compound: Cobalt (II) acetylacetone imide (200 mg.) |        |
| Target temp., °C                                    | 400    |
| Target material                                     | Quartz |
| Volatilization temp., °C                            | 287    |
| Pressure torr                                       | 730    |
| Hydrogen flow rate cc./min                          | 150    |

The deposit in this case consisted mainly of a bright, metallic foil, together with some black powdery material. Both deposits were identified as cobalt metal by X-ray diffraction analysis.

**EXAMPLE 10**

The compound trifluoroacetylacetone imide required in the preparation of the nickel derivative of Example 11, was synthesized as follows. Trifluoroacetylacetone (7.7 grams) was dissolved in 10 ml. absolute ethyl alcohol. Five ml. of concentrated aqueous  $\text{NH}_4\text{OH}$  and an additional 5 ml. ethyl alcohol were added successively. The mixture was heated briefly, nearly to boiling. After cooling, the mixture was then taken to dryness in a stream of nitrogen at room temperature. The residue was heated with 75 ml. N-heptane to give partial solution. The hot solution was filtered through filter paper and the insoluble residue remaining on the paper discarded. The filtrate was cooled and reduced to about  $\frac{1}{2}$  its original volume in a stream of nitrogen. After further cooling in a refrigerator the yellow crystals were filtered off, washed with cold petroleum ether and air dried at room temperature. Yield was 1.2 grams having a melting point of about 85-87 degree C.

**EXAMPLE 11**

The compound nickel (II) trifluoroacetylacetone imide (bis-2-imino-1,1,1-trifluoro-4-pentanonato nickel (II), for use as a metal-organic beta-ketoamine chelate vapor deposition plating compound was prepared as follows. Trifluoroacetylacetone imide, 1.07 grams, as prepared in Example 10, and dissolved in 10 ml. absolute ethyl alcohol was added to a suspension of 0.87 gram of nickel acetate tetrahydrate in 25 ml. absolute ethanol. One ml. of concentrated aqueous  $\text{NH}_4\text{OH}$  was added. The nickel acetate gradually went into solution upon heating and stirring. The solution was then cooled and reduced to about  $\frac{1}{3}$  of its original volume in a stream of nitrogen. Water (25 ml.) was then added to produce an immediate separation of red-tan precipitate. After the mixture had stood over

**10**

night at room temperature, the precipitate was filtered off, washed with water and dried in a vacuum to give 0.92 gram of light tan product (melting point about 198-199 degree C.). The product was recrystallized by dissolving it in 25 ml. warm absolute ethyl alcohol. The solution was filtered hot through filter paper and 25 ml. water was added to the filtrate. The tan precipitate was filtered off and dried in a vacuum at room temperature to give 0.60 gram of recrystallized product.

**EXAMPLE 12**

The results of chemical vapor deposition tests, using the aforescribed procedure and the apparatus of FIGS. 2 and 3 of this specification for nickel (II) trifluoroacetylacetone imide, as prepared in Example 11, are outlined in Table 6 below:

**TABLE 6**

|                                                         |        |
|---------------------------------------------------------|--------|
| Compound: Nickel trifluoroacetylacetone imide (200 mg.) |        |
| Target temp., °C                                        | 400    |
| Target material                                         | Quartz |
| Volatilization temp., °C                                | 287    |
| Pressure torr                                           | 730    |
| Hydrogen flow rate cc./min                              | 150    |

The metallic coating produced was identified as nickel metal by X-ray diffraction analysis.

**EXAMPLE 13**

The compound nickel acetylacetone-1,2-propylene diimide, for use as a metal-organic beta-ketoamine chelate vapor deposition plating compound was prepared as follows. Propylene diamine (3.7 grams) was added to 10 grams acetylacetone in a flask. After the exothermic reaction had subsided, the mixture was dissolved in 200 ml. of water. A solution of 0.05 mole of nickel acetate in 200 ml. water was added, followed by 100 ml. 1 molar aqueous  $\text{NH}_4\text{OH}$ . Upon heating, the resulting red solution gradually deposited red crystals. After 5 minutes heating, mixture was cooled, first to room temperature and then in a refrigerator. The compound was filtered off and air dried to give 8.1 grams of product. Recrystallization was achieved by dissolving in 50 ml. of hot methanol, filtering hot and adding 100 ml. water to the filtrate. Two successive recrystallization gave 6.0 grams of air dried red crystals of melting point about 158-159 degree C.

**EXAMPLE 14**

The results of chemical vapor deposition tests using the aforescribed procedure and the apparatus of FIGS. 2 and 3 of this specification for nickel acetylacetone-1,2-propylene-diimide, as prepared in Example 13 are outlined in Table 7 below.

**TABLE 7**

|                                                                 |  |
|-----------------------------------------------------------------|--|
| Compound: Nickel acetylacetone-1,2-propylene-diimide (200 mg.)— |  |
| Target temp., °C.—400                                           |  |
| Target material—Quartz                                          |  |
| Volatilization temp., °C.—287                                   |  |
| Pressure, torr—730                                              |  |
| Hydrogen flow rate, cc./min.—150                                |  |

In this case two bands of bright metallic deposit were formed, one upstream of the other. Both bands of metal foil were identified as pure nickel metal by X-ray diffraction analysis.

We claim as our invention:

1. A process of coating a substrate with metal comprising the steps of vaporizing a metal-organic beta-ketoamine chelate in a gaseous atmosphere and contacting a substrate, heated to a temperature higher than the vaporization temperature of the metal-organic beta-ketoamine chelate, with said vapor for a time sufficient to cause the substrate to be coated with metal.

## 11

2. The process of claim 1 wherein the metal-organic beta-ketoamine chelate has the structure



wherein M is selected from the group consisting of Ni, Cr, Cu, Co, Fe, Mn, Pd and Pt, R<sub>1</sub> is selected from the group consisting of CH<sub>3</sub> and CF<sub>3</sub>, R<sub>2</sub> is selected from the group consisting of CH<sub>3</sub> and CF<sub>3</sub>, R<sub>3</sub> is selected from the group consisting of H, CH<sub>3</sub> and CF<sub>3</sub>, X is selected from the group consisting of H and CH<sub>3</sub>, the gaseous atmosphere contains flowing hydrogen gas and the substrate temperature is between 200 and 700 degrees C.

3. The process of claim 1 wherein the metal-organic beta-ketoamine chelate has the structure



wherein M is selected from the group consisting of Ni, Cr, Cu, Co, Fe, Mn, Pd and Pt, R<sub>4</sub> is selected from the group consisting of CH<sub>3</sub> and CF<sub>3</sub>, R<sub>5</sub> is selected from

## 12

the group consisting of CH<sub>3</sub> and CF<sub>3</sub>, R<sub>6</sub> is selected from the group consisting of H, CH<sub>3</sub> and CF<sub>3</sub>, X is selected from the group consisting of H and CH<sub>3</sub>, the gaseous atmosphere contains flowing hydrogen gas and the substrate temperature is between 200 and 700 degrees C.

5 4. The process of claim 1 wherein the substrate is a fibrous material.

5 5. The process of claim 1 wherein the metal-organic beta-ketoamine chelate is selected from the group consisting of bisacetylacetoneimide nickel (II), bisacetylacetone-ethylenediimino nickel (II) and bisacetylacetoneethylenediimino copper (II), the gaseous atmosphere contains flowing hydrogen gas and the substrate temperature is between 200 and 700 degrees C.

15 6. The process of claim 5 wherein the hydrogen gas is flowing at a rate of at least 60 c./min., and gaseous by products of vaporization are removed.

## References Cited

## UNITED STATES PATENTS

|           |         |                 |       |           |
|-----------|---------|-----------------|-------|-----------|
| 3,356,527 | 12/1967 | Moshier et al.  | ----- | 117—107.2 |
| 3,242,102 | 3/1966  | Schneckenbecker | ---   | 117—107.2 |
| 2,430,520 | 11/1947 | Marboe          | ----- | 117—107.2 |

25 ALFRED L. LEAVITT, Primary Examiner

W. E. BALL, Assistant Examiner

U.S. Cl. X.R.

260—439